

Aug. 9, 1966

J. F. BALDWIN ET AL  
ALLOYS FOR HIGH TEMPERATURE USE CONTAINING  
CHROMIUM, TUNGSTEN, NICKEL, COBALT  
Filed April 3, 1964

3,265,494



FIG. 1



FIG. 2



FIG. 3



FIG. 4

1

3,265,494

## ALLOYS FOR HIGH TEMPERATURE USE CONTAINING CHROMIUM, TUNGSTEN, NICKEL, COBALT

James F. Baldwin, Locust Valley, N.Y., and Arthur T. Cape, Monterey, Calif., assignors to Coast Metals, Inc., Little Ferry, N.J., a corporation of Delaware

Filed Apr. 3, 1964, Ser. No. 357,124

2 Claims. (Cl. 75—171)

This application is a continuation-in-part of application Serial No. 125,355 filed July 20, 1961, which was a continuation-in-part of application Serial No. 766,674 filed October 13, 1958, both of which are now abandoned.

This invention relates generally to alloys for high temperature use, containing cobalt, chromium, tungsten and nickel as their principal constituents.

In U.S. Patent No. 2,801,165, there is disclosed a cobalt-base alloy which contains 18.75-23.25% tungsten, and 26-30% chromium, but which is substantially free from nickel. This alloy has a short time tensile strength, at 1800° F., of about 40,000 p.s.i.

In U.S. Patent No. 2,684,299, there is disclosed a cobalt-base alloy containing 16-20% tungsten and 7-12% nickel, but this alloy, of which a typical example is the alloy commonly known as Haynes Stellite No. 36, has a maximum short time tensile strength, at 1800° F., of about 40,000 p.s.i.

We have discovered, however, that by utilizing an alloy having a composition within the following ranges, and provided that the ratio of cobalt to chromium in the alloy is always at least 1.4:1, that the short time tensile strength of the alloy, at 1800° F., is increased to a minimum of 48,000 p.s.i.

|           | Range, percent | Preferred, percent |
|-----------|----------------|--------------------|
| Carbon    | 0.7-1.0        | 0.85               |
| Chromium  | 26-30          | 28                 |
| Tungsten  | 18-21          | 19.5               |
| Nickel    | 4.0-6.0        | 5.0                |
| Boron     | .005-.1        | .2                 |
| Silicon   | 1.00 Max.      | .1                 |
| Manganese | 1.00 Max.      | .9                 |
| Vanadium  | .75-.1.25      | .4                 |
| Iron      | 3.0 Max.       | 45.00              |
| Cobalt    | Balance        |                    |

If a maximum of chromium is used in the alloy, the minimum amount of cobalt which can be used in the alloy, in order to maintain the aforesaid minimum ratio of cobalt to chromium, would be 42%. If the minimum amount of chromium is used in the alloy, the minimum amount of cobalt which can be used in the alloy, in order to maintain the aforesaid minimum ratio of cobalt to chromium, would be 36.4%. As a practical matter, therefore, the cobalt range of such an alloy would vary from 36.4 to 42%, although the cobalt content could be increased beyond this range, depending upon the quantities of the other ingredients present in the alloy, principally the amounts of tungsten and nickel.

Moreover, it has been found that maximum values as to short time tensile strength are maintained by decreasing the tungsten content of the alloy as the nickel content is increased.

The alloys of the aforesaid Patents 2,801,165 and 2,684,299, have, as already stated, a short time tensile strength, at 1800° F., of about 40,000 p.s.i. In contrast to this, the alloys of the present invention have a short time tensile strength, at 1800° F., of a minimum of 48,000 p.s.i. This increase of at least 20% in the short time tensile strength is unusual in view of the relatively small amount of nickel in the alloy, and is probably due to the use of the relatively high chromium content in conjunction

2

with the small amount of nickel. In any event, the difference in short time tensile strength is obviously a difference in degree rather than kind.

The nickel range of 4 to 6% is, however, extremely critical from another viewpoint, and that is, from the viewpoint of ductility or freedom from brittleness of the alloy.

This may be explained by reference to the accompanying photomicrographs, in which

FIG. 1 is a photomicrograph, at a magnification of 270 $\times$ , of an alloy corresponding to the above-mentioned "preferred" alloy, but containing 10% nickel and 40% cobalt;

FIG. 2 is a photomicrograph, at a magnification of 270 $\times$ , of an alloy corresponding to the above-mentioned "preferred" alloy, but containing 7% nickel and 43% cobalt;

FIG. 3 is a photomicrograph, at a magnification of 270 $\times$ , of an alloy corresponding to the "preferred" alloy, and

FIG. 4 is a photomicrograph, at a magnification of 270 $\times$ , of an alloy corresponding to the "preferred" alloy, but containing 3% nickel and 47% cobalt.

Referring to FIG. 1, it will be seen that there is an excessive amount of a continuous black or dark phase, which is an acicular carbide, and which, although it supplies resistance to wear in the alloy, is highly disadvantageous in that it is a source of brittleness in the alloy.

This brittleness, which makes the alloy undesirable both for hard facing purposes and for making castings thereof, manifests itself in the following rather dramatic manner. Weld rods made of the alloy were passed through a centerless grinder for the purpose of grinding the rods to make them suitable for purposes of welding. Due to the brittleness of the rods virtually all of the rods became shattered in the course of their passage through the centerless grinder.

Referring to FIG. 2, it will be seen that the black or dark phase of the alloy, while slightly less in amount, is still substantial and continuous, to the extent that this alloy was also brittle, and the great majority of rods of this analysis passed through the centerless grinder became shattered in the course of their passage through the grinder.

Referring to FIG. 3, it will be seen that there is a dark phase which is substantially less in area than the dark phase in FIGS. 1 and 2. This alloy was entirely free from brittleness, exhibited a high degree of ductility, and 100% of the rods of this analysis were passed through the centerless grinder without any sign of shattering.

Referring to FIG. 4, it will be seen that there is a gray phase, similar in total area to the dark phase in FIG. 2, but in which a fine precipitate is formed which causes an increase in hardness, which, in turn, causes the alloy as a whole to have less resistance to impact than the alloy of FIG. 3. Such an alloy, while ductile, is undesirable for manufacture into weld rods and castings, because of this increase in hardness and resulting brittleness.

The distinction between the alloys of FIGS. 1, 2, 3 and 4 were further emphasized in testing the alloys with a Knoop indenter, using a 200 gm. load. The difference in Knoop values appears in the following table:

| Alloy: | Knoop value |
|--------|-------------|
| FIG. 1 | 535         |
| FIG. 2 | 738         |
| FIG. 3 | 678         |
| FIG. 4 | 704         |

These Knoop values are a further indication of the suitability or adaptability of the alloys for use as weld rods and small castings. As apparent from the table, the Knoop value of the alloy with 10% nickel was too

low. With 7% nickel, the Knoop value was too high. With 5% nickel, the Knoop value was at an optimum. With 3% nickel, the Knoop value rose to an undesirable point. The indication, therefore, was that the desired range of nickel in the alloy extends from a point somewhat below 7% to a point somewhat above 3%.

Based on all of the foregoing tests and results, it was concluded that optimum results, from the standpoint of a combination of ductility (freedom from brittleness), and wear resistance, were obtained in the rather narrow and critical range of 4 to 6% nickel.

In application, Serial No. 766,674, examples of alloys were disclosed containing in excess of about 6% nickel, specifically, nickel in amounts of 10%, and it was stated that these alloys had short time tensile strengths of about 54,000 p.s.i. However, as apparent from the foregoing photomicrographs and the tests described relative thereto, the alloys in Serial No. 766,674, containing 10% nickel, would not be suitable for manufacture into weld rods or for castings and would be entirely unsatisfactory for hard facing purposes, due to their brittleness or lack of ductility.

The alloys of the present invention are particularly useful for the joining areas of Waspalloy jet engine turbine blades, where constant hammering takes place at the joining areas of the interlocking blades. It is obvious that any brittleness in the alloy would render it entirely unsatisfactory for this purpose.

It may be further pointed out that in application, Serial No. 766,674, it was stated that in order to obtain high strengths with ductility, and avoid brittleness in the alloy, it was necessary to decrease the nickel as the chromium content increased. In the examples, wherein the nickel content was 10%, the chromium content was 19%, or far below the 26-30% range of chromium in the alloy of the present invention. The alloy of the present inven-

tion is accordingly distinguished from the alloy of Patent No. 2,684,299, not only in its high chromium range, but in its narrow and critical nickel range.

Having thus described our invention, we claim:

1. An alloy especially adapted for use as a welding material at high temperatures, said alloy consisting of carbon 0.7 to 1.0%, chromium 26 to 30%, tungsten 18 to 21%, nickel 4 to 6%, boron 0.005 to 0.1%, 0 to 1% silicon, 0 to 1% manganese, 0 to 3% iron, 0.75 to 1.25% vanadium, and the balance being essentially all cobalt, and the ratio of cobalt to chromium being always at least 1.4 to 1, said alloy having a ductility and freedom from brittleness such that rods of said alloy may be passed through a centerless grinder without the shattering of any substantial percentage thereof.

2. An alloy especially adapted for use as a welding material at high temperatures, said alloy consisting of about 0.85% carbon, about 28% chromium, about 19.5% tungsten, about 5% nickel, about .05% boron, about 0.2% silicon, about 0.1% manganese, about .9% vanadium, about .4% iron, and about 45% cobalt, said alloy having a ductility and freedom from brittleness such that rods of said alloy may be passed through a centerless grinder without the shattering of any substantial percentage thereof.

#### References Cited by the Examiner

#### UNITED STATES PATENTS

|           |        |                |       |        |
|-----------|--------|----------------|-------|--------|
| 2,684,299 | 7/1954 | Binder         | ----- | 75—171 |
| 2,801,165 | 7/1957 | Baldwin et al. | ----- | 75—171 |

HYLAND BIZOT, Primary Examiner.

DAVID L. RECK, Examiner.

R. O. DEAN, Assistant Examiner.